# EUROPEAN PATENT APPLICATION

(11) **EP 0 740 204 A1**
(43) Date of publication of application: **30.10.1996**
(21) Application number: 96420133.9
(22) Date of filing: 18.04.1996
(51) Int. Cl.: G03C 7/30

(54) **Photographic elements containing magenta dye forming couplers and fade reducing compounds--N**

(30) Priority: 26.04.1995 US 428981
(71) Applicant: EASTMAN KODAK COMPANY, Rochester, New York 14650-2201 (US)
(72) Inventor: Jain, Rakesh, c/o Eastman Kodak Company, Rochester, New York 14650-2201 (US)
(74) Representative: Fevrier, Murielle Françoise E.

(57) **Abstract**

Dye fade in photographic images prepared from a silver halide photographic element having a light sensitive silver halide emulsion layer and a pyrazoloazole dye forming coupler is reduced by using a combination of stabilizer compounds as shown in the specification.

## Description

### Field of the Invention

This invention relates to photographic elements containing particular magenta dye forming couplers associated with compounds which reduce fading of the dyes formed from the couplers on processing of the photographic element.

### Background of the Invention

In a silver halide photographic element, a color image is formed when the element is exposed to light and then subjected to color development with a primary aromatic amine developer. Color development results in imagewise reduction of silver halide and production of oxidized developer. Oxidized developer reacts with one or more incorporated dye-forming couplers to form an imagewise distribution of dye.

The dyes that are formed by any color coupler during processing have a tendency to fade over time as a result of exposure to light, heat and humidity. As all three image dyes of a typical color element fade, this results in overall fading of the image over time. In addition, since the three image dyes may not fade at the same rate, an apparent change in image color may result. Such change is particularly noticable in the case of magenta image dye fading.

A variety of magenta dye-forming coupler types have been used in photographic materials. Among the known magenta dye-forming couplers are cyclic azoles such as pyrazolotriazoles, pyrazolobenzimidazoles, and imidazopyrazoles. These couplers contain bridgehead nitrogen 5,5 fused ring systems and include such couplers as pyrrolo[1,2-b]pyrazoles, pyrazolo[3,2-c] [1,2,4] triazoles, pyrazolo[2,3-b][1,2,4]triazoles, imidazo[1,2-b]pyrazoles, imidazo[1,5-b]pyrazoles, imidazo[1,2-a]imidazoles, imidazo[1,2-b][1,2,4] triazoles, imidazo[2,1-c][1,2,4]triazoles, imidazo[5,1-c][1,2,4]triazoles and [1,2,4]triazolo[3,4-c][1,2,4]triazole.

A significant disadvantage of pyrazoloazole couplers is fading of the dyes formed from them by photographic processing due to extended exposure to low levels of light. Compounds which are included in photographic elements to reduce image dye fading are known as stabilizers. Inclusion of stabilizers in color photographic materials can reduce the deterioration of the dye images which occurs over time as a result of the action of light, heat or humidity. This is true for dyes formed from pyrazoloazole couplers. US Patents 5,236,819 and 5,082,766 describe the use of certain stabilizers with pyrazoloazole couplers to improve their dye stability. However, it would be desirable to further improve the light stability of dyes derived from cyclic azole magenta dye forming couplers, and thus retain the color rendition of the image for a longer period of time.

### Summary of the Invention

We have found that highly stable magenta dye images formed from cyclic azole magenta couplers can be obtained if there is associated with the coupler a combination stabilizer compounds R, S and N, shown below.

The present invention therefore provides a silver halide photographic element comprising a support bearing a light sensitive silver halide emulsion layer and a cyclic azole magenta dye forming coupler associated with a stabilizer combination comprising:
i) a compound having the following Formula R:
ii) a compound having the following Formula S: and
iii) a compound having the following Formula N: wherein:
   each R₁ independently represents a hydrogen atom, an alkyl group, an alkenyl group or an aryl group;
   each R₂ independently represents a halogen atom, an alkyl group, an alkenyl group an alkoxy group, an aryl group, an aryloxy group, an alkylthio group, an aryl thio group, an acyl group, an an acylamino group, a sulfonyl group, a sulfonamide group or a hydroxy group;
   each m is, individually an integer of 0 to 4;
   A represents an alkylene group having 1 to 6 carbon atoms in its linear structure;
   R₃ represents an aryl group or a heterocyclic group;
   Z₁ and Z₂ each represent an alkylene group having 1 to 3 carbon atoms provided that the total number of carbon atoms in the ring is 3 to 6;
   n is an integer of 1 or 2;
   M is Cu, Co, Ni, Pd or Pt;
   each W², W³, W⁴ and W⁵ are, independently, hydrogen, halogen, nitro, cyano, alkyl, aryl, alkoxy, aryloxy, carbonyl, sulfonyl, amido, carbamoyl, sulfonamido, sulfamoyl or heterocyclyl, or any of W², W³, W⁴ and W⁵ may together form a cycloalkyl or heterocyclic group;
   each W⁶ and W⁷ are, independently hydrogen, hydroxy alkyl or aryl, or W⁶ and W⁷ ,together, can form a 5 or 6 membered ring.

Photographic elements of the present invention yield magenta dye images that have low fading when exposed to light.

### Detailed Description of the Invention

As used herein, unless otherwise indicated the alkyl and aryl groups, and the alkyl and aryl portions of groups, can be unsubstituted or substituted with non-interfering substituents. Typical alkyl groups have 1 to 32 carbon atoms and typical aryl groups have 6 to 32 carbon atoms. Depending upon the position of the group, preferred alkyl groups can have 1 to 20 carbon atom, 1 to 12 carbon atoms or 1 to 4 carbon atoms and preferred aryl groups can have 6 to 20 or 6 to 10 carbon atoms. Other groups identified below which contain a replacable hydrogen atom can be substituted or not, depending on the particular structure and properties desired.

The magenta dye forming couplers of this invention can be based on any of the bridgehead nitrogen 5,5 fused ring system identified above. Preferred couplers are pyrazolotriazoles represented by Formula II: wherein:
R₆ is hydrogen or a substituent;
R₇ is a ballast group; and
X is hydrogen or a coupling-off-group; and
Zₐ, Z_{b}, and Z_{c} are independently a substituted or
unsubstituted methine group, =N-, or -NH-, provided that one of either the Zₐ-Z_{b} bond or the Z_{b}-Z_{c} bond is a double bond and the other is a single bond, and when the Z_{b}-Z_{c} bond is a carbon-carbon double bond, it can be part of the aromatic ring and at least one of Zₐ, Z_{b}, and Z_{c} represents a methine group connected to R₇.

Preferred pyrazolotriazole couplers of this invention are 1H-pyrazolo[2,3-b][1,2,4]triazoles represented by Formula III: wherein:
X, R₆ and R₇ are as previously defined.

Examples of suitable R₆ groups are alkyl, which can be straight or branched, such as methyl, ethyl, n-propyl, n-butyl, t-butyl, trifluoromethyl, tridecyl or 3-(2,4-di-t-amylphenoxy)propyl; alkoxy, such as methoxy or ethoxy; alkylthio, such as methylthio or octylthio; aryl, aryloxy or arylthio, such as phenyl, 4-t-butylphenyl, 2,4,6-trimethylphenyl, phenoxy, 2-methylphenoxy, phenylthio or 2-butoxy-5-t-octylphenylthio; heterocyclyl, heterocyclyloxy or heterocyclylthio, each of which contain a 3 to 7 membered heterocyclic ring composed of carbon atoms and at least one hetero atom selected from oxygen, nitrogen and sulfur, such as 2-furyl, 2-thienyl, 2-benzimidazolyloxy or 2-benzothiazolyl; cyano; acyloxy, such as acetoxy or hexadecanoyloxy; carbamoyloxy, such as N-phenylcarbamoyloxy or N-ethylcarbamoyloxy; silyloxy, such as trimethylsilyloxy; sulfonyloxy, such as dodecylsulfonyloxy; acylamino, such as acetamido or benzamido; anilino, such as phenylanilino or 2-chloroanilino; ureido, such as phenylureido or methylureido; imido, such as N-succinimido or 3-benzylhydantoinyl; sulfamoylamino, such as N,N-dipropyl-sulfamoylamino or N- methyl-N-decylsulfamoylamino; carbamoylamino, such as N-butylcarbamoylamino or N,N-dimethylcarbamoylamino; alkoxycarbonylamino, such as methoxycarbonylamino or tetradecyloxycarbonylamino; aryloxycarbonylamino, such as phenoxycaronylamino, 2,4-di-t-butylphenoxycarbonylamino; sulfonamido, such as methanesulfonamido or hexadecanesulfonamido; carbamoyl group, such as N-ethylcarbamoyl or N,N-dibutylcarbamoyl; acyl, such as acetyl or (2,4-di-t-amylphenoxy)acetyl; sulfamoyl, such as N-ethylsulfamoyl or N,N-dipropylsulfamoyl; sulfonyl, such as methanesulfonyl or octanesulfonyl; sulfinyl, such as octanesulfinyl or dodecylsulfinyl; alkoxycarbonyl, such as methoxycarbonyl or butyloxycarbonyl; aryloxycarbonyl, such as phenyloxycarbonyl or 3-pentadecyloxycarbonyl; alkenyl; hydroxyl; amino; and carbonamido groups.

Preferably, R₆ represents a tertiary alkyl group of 4 to 12 carbon atoms. Most preferably it represents t-butyl.

The ballast group represented by R₇ is a group of such size and configuration that, in combination with the remainder of the molecule, it provides the coupler, and the dye formed from it, with sufficient bulk that it is substantially non-diffusible from the layer in which it is coated in the photographic element. Representative ballast groups include alkyl or aryl groups containing 6 to 32 carbon atoms. Other ballast groups include alkoxy, aryloxy, arylthio, alkylthio, alkoxycarbonyl, aryloxycarbonyl, carboxy, acyl, acyloxy, carbonamido, carbamoyl, alkylcarbonyl, arylcarbonyl, alkysulfonyl, arylsulfonyl, sulfamoyl, sulfenamoyl, alkylsulfinyl, arylsulfinyl, alkylphosphonyl, arylphosphonyl, alkoxyphosphonyl, and arylphosphonyl. Preferably R₇ is an alkyl group of 6 to 32 carbon atoms

Possible substituents for R₆ and R₇ include halogen, alkyl, aryl, aryloxy, heterocyclyl, cyano, alkoxy, acyloxy, carbamoyloxy, silyloxy, sulfonyloxy, acylamino, anilino, ureido, imido, sulfonylamino, carbamoylamino, alkylthio, arylthio, heterocyclylthio, alkoxycarbonylamino, aryloxycarbonylamino, sulfonamido, carbamoyl, acyl, sulfamoyl, sulfonyl, sulfinyl, alkoxycarbonyl, aryloxycarbonyl, alkenyl, carboxyl, sulfo, hydroxyl, amino and carbonamido groups.

The coupling off group represented by X can be a hydrogen atom or any of the coupling-off groups known in the art. Coupling-off groups can determine the equivalency of the coupler, can modify the reactivity of the coupler, or can advantageously affect the layer in which the coupler is coated or other layers in the element by performing, after the release from the coupler, such functions as development inhibition, development acceleration, bleach inhibition, bleach acceleration, color correction, and the like. Representative classes of coupling-off groups include halogen, particularly chlorine, bromine, or fluorine, alkoxy, aryloxy, heterocyclyloxy, heterocyclic, such as hydantoin and pyrazolo groups, sulfonyloxy, acyloxy, carbonamido, imido, acyl, heterocyclythio, sulfonamido, alkylthio, arylthio, heterocyclythio, sulfonamido, phosphonyloxy, and arylazo.

preferably, X is hydrogen or halogen. Most preferably X is hydrogen or chlorine.

Specific couplers within the scope of the present invention have the following structures:

The stabilizers that have the Formula R, above, are believed to stabilize the dye image by scavenging free radicals. In this formula, the group represented by A is a straight, branched or cyclic alkylene group, the linear portion of which has 1 to 6 carbon atoms, which can be substitituted with one or more aryl, cyano, halogen, heterocyclyl, cycloalkyl, alkoxy, hydroxy, and aryloxy groups. The alkylene group can form a cycloalkyl ring, such as

In Formula R, each R₁ can be a group as defined above for R₆ or R₇ in Formula III. These include halogen, alkyl, cycloalkyl, alkenyl, alkoxy, aryl, aryloxy, alkylthio, arylthio, acyl, acylamino, sulfonyl and sulfonamido.

Preferred compounds represented by Formula R, are those in which:
each R₁ independently is hydrogen, alkyl or cycloalkyl of 1 to 8 carbon atoms;
each R₂ is independently hydrogen, hydroxy, alkyl or alkoxy of 1 to 8 carbon atoms;
each m is an integers of 0 to 2; and
A is an alkylene group of 1 to 10 carbon atoms.

Representative examples of stabilizer compounds which satisfy Formula R are:

The stabilizers that have the Formula S, above are believe to stabilize by acting as singlet oxygen quenchers. In this formula the aryl and heterocyclic group represented by R₃ include phenyl, 1-naphthyl, 2-furyl and 2-thienyl. They can be substituted with groups described above in Formula III for R₆, as can be the alkylene groups represented by Z₁ and Z₂.

Preferred stabilizers represented by Formula S, are those having the following Formula S1: wherein:
R₈ represents alkyl, alkoxy, alkylthio, amido, ureido, or halogen;
R₉ is alkyl;
r is an integer of 1 or 2; and
s is an integer of 0 to 4.

Representative examples of stabilizer having the Formula S are:

The stabilizers of Formula N, above, are known compounds and have been known to act as stabilizers for dyes derived from couplers in photographic elements. They are described in EP Published Application 0 618 497, published October 5, 1994, and in US Patents 4,906,559, issued March 6, 1990 and 5,208,140, issued May 4, 1993. As described in these patents, these compounds act as singlet oxygen quenchers and are used in amounts that give the layer in which they are coated a noticable color. However, these compounds have not been used in combination with other magenta dye stabilizers having structures R and S, shown above. Nor, has it been suggested that, when so used, they would enhanced the stabilization effect of another singlet oxygen quencher, the S compound shown above. When used in this way, the N stabilizers can be used in small enough amounts that they do not give the layer in which they are coated an objectionable color.

In a preferred embodiment, in Formula N, each of W², W³, W⁴, W⁵, W⁶ and W⁷ are hydrogen, halogen, alkyl or alkoxy having more than 20 carbon atoms (further preferably no more than 12). Any of W², W³, W⁴, W⁵, W⁶ and W⁷ can independently be methyl, ethyl, propyl, butyl, pentyl, octyl or can be the corresponding alkoxy analogue.

Particular examples of stabilizers of formula N include the following:

Compounds of Formula N can be synthesized as described in EP Published Application 0 618 497, referred to above.

Typically, the couplers and the stabilizers with which they are associated are dispersed in the same layer of the photographic element in a high boiling organic compound known in the art as a coupler solvent. Representative coupler solvents include phthalic acid alkyl esters such as dibutyl phthalate and dioctyl phthalate, phosphoric acid esters such as tricresyl phosphate, diphenyl phosphate, tris-2-ethylhexyl phosphate, and tris-3,5,5-trimethylhexyl phosphate, citric acid esters such as tributyl acetylcitrate, benzoic acid esters such as octyl benzoate, aliphatic amides such as N,N-diethyl lauramide, and alkyl phenols such as 2,4-di-t-butyl phenol. Especially preferred coupler solvents are the phthalate esters, which can be used alone or in combination with one another or with other coupler solvents. Selection of the correct coupler solvent has been found to have an influence both on the hue of the dye formed on coupling as well as on its stability.

Throughout this application a reference to any type of chemical "group" includes both the unsubstituted and substituted forms of the group described. Generally, unless otherwise specifically stated, substituent groups usable on molecules herein include any groups, whether substituted or unsubstituted, which do not destroy properties necessary for the photographic utility. It will also be understood throughout this application that reference to a compound of a particular general formula includes those compounds of other more specific formula which specific formula falls within the general formula definition. Examples of substituents on any of the mentioned groups can include known substituents, such as: halogen, for example, chloro, fluoro, bromo, iodo; alkoxy, particularly those with 1 to 6 carbon atoms (for example, methoxy, ethoxy); substituted or unsubstituted alkyl, particularly lower alkyl (for example, methyl, trifluoromethyl); alkenyl or thioalkyl (for example, methylthio or ethylthio), particularly either of those with 1 to 6 carbon atoms; substituted and unsubstituted aryl, particularly those having from 6 to 20 carbon atoms (for example, phenyl); and substituted or unsubstituted heteroaryl, particularly those having a 5 or 6-membered ring containing 1 to 3 heteroatoms selected from N, O, or S (for example, pyridyl, thienyl, furyl, pyrrolyl); and others known in the art. Alkyl substituents may specifically include "lower alkyl", that is having from 1 to 6 carbon atoms, for example, methyl, ethyl, and the like. Further, with regard to any alkyl group, alkylene group or alkenyl group, it will be understood that these can be branched or unbranched and include ring structures.

The coupler and stabilizer compounds of the present invention are known compounds and can be prepared by techniques known to those skilled in the art. References which describe the preparation of the magenta dye forming couplers are the patents and published applications referred to above as describing these compounds, and references cited therein. The preparation of Stabilizer Compounds R and S is described in US Patent 5,236,819 and references cited therein. The synthesis of Stabilizer Compound N is easily accomplished by methods known to those skilled in the art, such as by reacting a suitably substituted amine with an activated alkene, for example, with acrylonitrile.

Typically the amount of each of compound R and compound S will range from about 0.2 to about 3.0 moles stabilizer per mole of coupler, preferably from about 0.5 to 1.5 moles stabilizer per mole of coupler. The amount of compound N will range from about 0.01 to 0.5 moles stabilizer per mole of coupler, preferably preferably from about 0.02 to 0.1 moles stabilizer per mole coupler.

The pyrazoloazole coupler, is typically coated in the element at a coverage of from 0.25 mmol/m² to 1.0 mmol/m², and preferably at a coverage of from 0.40 to 0.70 mmol/m². When a coupler solvent is employed, it typically is present in an amount of 0.50 to 5.0 mg. per mg. coupler, and preferably in an amount of 1.0 to 3.0 mg. per mg. coupler.

The photographic elements of this invention can be black and white elements (for example, using magenta, cyan and yellow dye forming couplers), single color elements or multicolor elements. Multicolor elements contain dye image-forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

Photographic elements of this invention can have the structures, components, exposure and processing shown on Research Disclosure, February 1995, Item 37038, pages 79-114. Research Disclosure is published by Kenneth Mason Publications, Ltd., Dudley Annex, 12a North Street, Emsworth, Hampshire P010 7DQ, ENGLAND. Specific elements can be those shown on pages 96-98 of this Research Disclosure item as Color Paper Elements 1 and 2, in which is employed in the magenta dye forming layers the stabilizer combinations of the the present invention instead of the stabilizers shown there. A typical multicolor photographic element of this invention comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like. All of these can be coated on a support which can be transparent or reflective (for example, a paper support). Photographic elements of the present invention may also usefully include a magnetic recording material as described in Research Disclosure, Item 34390, November 1992, or a transparent magnetic recording layer such as a layer containing magnetic particles on the underside of a transparent support as in US 4,279,945 and US 4,302,523. The element typically will have a total thickness (excluding the support) of from 5 to 30 microns. While the order of the color sensitive layers can be varied, they will normally be red-sensitive, green-sensitive and blue-sensitive, in that order on a transparent support, (that is, blue sensitive furthest from the support) and the reverse order on a reflective support being typical.

This invention also contemplates the use of photographic elements of the present invention in what are often referred to as single use cameras (or "film with lens" units). These cameras are sold with film preloaded in them and the entire camera is returned to a processor with the exposed film remaining inside the camera. Such cameras may have glass or plastic lenses through which the photographic element is exposed.

The stabilizers of this invention can be used in photographic elements that are intended to be processed in amplification processes that use developer/amplifier solutions described in USPatent 5,324,624, for example. When processed in this way, the low volume, thin tank processing system and apparatus described in USPatent Application 08/221,711, filed March 31, 1994, preferably is employed.

The following examples further illustrate this invention.

### Example 1

### Photographic Evaluation

Dispersions of the coupler and stabilizers were prepared in the following manner. In one vessel there was combined coupler, coupler solvents, stabilizer(s), and ethyl acetate and the combination was warmed to dissolve. In a second vessel, the gelatin, surfactant (Alkanol XC™ from E.I. duPont Co.) and water were combined and passed three times through a Gaulin colloid mill. The ethyl acetate was removed by evaporation and water was added to restore the original weight after milling.

Photographic elements were prepared by coating the following layers in the order listed on a resin-coated paper support:

### 1st layer

| | |
|---|---|
| Gelatin | 3.23 g/m² |

### 2nd layer

| | |
|---|---|
| Gelatin | 1.61 g/m² |
| Coupler M-9 | 0.22 g/m² |
| Dibutyl phthalate coupler solvent | 0.16 g/m² |
| Diethylhexyl phthalate coupler solvent | 0.16 g/m² |
| Stabilizer R-4 | 0.18 g/m² |
| Stabilizer S-8 | 0.18 g/m² |
| Stabilizer N-15 | 0.02 g/m² |
| Green sensitized AgCl emulsion | 0.17 g/m² |

### 3rd layer

| | |
|---|---|
| Gelatin | 1.34 g/m² |
| 2-(2H-benzotriazol-2-yl)-4,6-bis-(1,1-dimethylpropyl)phenol | 0.73 g/m² |
| Tinuvin 326^{TM} (Ciba-Geigy) | 0.13 g/m² |

### 4th layer

| | |
|---|---|
| Gelatin | 1.40 g/m² |
| Bis(vinylsulfonylmethyl)ether | 0.14 g/m² |

The photographic elements were given stepwise exposures to green light and processed at 35°C as follows:

| | |
|---|---|
| Developer | 45 sec. |
| Bleach-Fix | 45 sec. |
| Wash (running water) | 1 min.30 sec. |

The developer and bleach-fix had the following compositions:

### Developer

| | |
|---|---|
| Water | 700.00 mL |
| Triethanolamine | 12.41 g |
| Blankophor REU^{TM} (Mobay Corp.) | 2.30 g |
| Lithium polystyrene sulfonate (30%) | 0.30 g |
| N,N-Diethylhydroxylamine (85%) | 5.40 g |
| Lithium sulfate | 2.70 g |
| N-{2-[(4-amino-3-methylphenyl) ethylamino]ethyl}methanesulfonamide sesquisulfate | 5.00 g |
| 1-Hydroxyethyl-1,1-diphosphonic acid (60%) | 0.81 g |
| Potassium carbonate, anhydrous | 21.16 g |
| Potassium chloride | 1.60 g |
| Potassium bromide | 7.00 mg |
| Water to make | 1.00 L |
| pH @ 26.7 °C adjusted to 10.04 +/- 0.05 | |

### Bleach-Fix

| | |
|---|---|
| Water | 700.00 mL |
| Solution of ammonium thiosulfate (54.4%) + ammonium sulfite (4%) | 127.40 g |
| Sodium metabisulfite | 10.00 g |
| Acetic acid (glacial) | 10.20 g |
| Solution of ammonium ferric ethylenediaminetetraacetate (44%) + ethylenediaminetetraacetic acid (3.5%) | 110.40 g |
| Water to make | 1.00 L |
| pH @ 26.7 °C adjusted to 5.5 ± 0.1 | |

Magenta dyes were formed upon processing. The following photographic characteristics were determined:
Dₘₐₓ (the maximum density to green light);
Speed (the relative log exposure required to yield a density to green light of 1.0);
Contrast (the ratio (S-T)/0.6, where S is the density at a log exposure 0.3 units greater than the Speed value and T is the density at a log exposure 0.3 units less than the Speed value).

Elements which had been exposed and processed to provide a Status A green density of 1.0 and 1.7 were irradiated with a 50 klux high intensity daylight (HID) for 3 weeks. The change in density as a result of irradiation was measured at the end of 3 weeks or at the end of 2 weeks and again at the end of 3 weeks. This data shows that the stabilizer combinations of this invention provide an improvement in the light stability compared with a combination that does not contain Stabilizer N.

### Example 2

Example 1 was repeated, except that the amount of Stabilizer compound N-15 was used at two different levels and the composition of the 2nd layer was as follows:

### 2nd layer

| | |
|---|---|
| Gelatin | 1.61 g/m² |
| Coupler M-9 | 0.22 g/m² |
| Dibutyl phthalate coupler solvent | 0.24 g/m² |
| Diethylhexyl phthalate coupler solvent | 0.24 g/m² |
| Stabilizer R-4 | 0.13 g/m² |
| Stabilizer S-2 | 0.13 g/m² |
| Stabilizer N-15 | see table |
| Green sensitized AgCl emulsion | 0.17 g/m² |

The light fade data are shown in Table II.

## Claims

1. A silver halide photographic element comprising a support bearing a light sensitive silver halide emulsion layer and a cyclic azole magenta dye forming coupler associated with a stabilizer combination comprising:
i) a compound having the following Formula R:
ii) a compound having the following Formula S: and
iii) a compound having the following Formula N: wherein:
each R₁ independently represents a hydrogen atom, an alkyl group, an alkenyl group or an aryl group;
each R₂ independently represents a halogen atom, an alkyl group, an alkenyl group an alkoxy group, an aryl group, an aryloxy group, an alkylthio group, an aryl thio group, an acyl group, an an acylamino group, a sulfonyl group, a sulfonamide group or a hydroxy group;
each m is, individually an integer of 0 to 4;
A represents an alkylene group having 1 to 6 carbon atoms in its linear structure;
R₃ represents an aryl group or a heterocyclic group;
Z₁ and Z₂ each represent an alkylene group having 1 to 3 carbon atoms provided that the total number of carbon atoms in the ring is 3 to 6;
n is an integer of 1 or 2;
M is Cu, Co, Ni, Pd or Pt;
each W², W³, W⁴ and W⁵ are, independently, hydrogen, halogen, nitro, cyano, alkyl, aryl, alkoxy, aryloxy, carbonyl, sulfonyl, amido, carbamoyl, sulfonamido, sulfamoyl or heterocyclyl, or any of W², W³, W⁴ and W⁵ may together form a cycloalkyl or heterocyclic group;
each W⁶ and W⁷ are, independently hydrogen, hydroxy alkyl or aryl, or W⁶ and W⁷ ,together, can form a 5 or 6 membered ring.

2. A photographic element of claim 1, wherein the magenta dye forming coupler has the structure: wherein:
R₆ is hydrogen or a substituent;
R₇ is a ballast group; and
X is hydrogen or a coupling-off-group; and
Zₐ, Z_{b}, and Z_{c} are independently a substituted or
unsubstituted methine group, =N-, or -NH-, provided that one of either the Zₐ-Z_{b} bond or the Z_{b}-Z_{c} bond is a double bond and the other is a single bond, and when the Z_{b}-Z_{c} bond is a carbon-carbon double bond, it can be part of the aromatic ring and at least one of Zₐ, Z_{b}, and Z_{c} represents a methine group connected to R₇.

3. A photographic element of claim 2, wherein the magenta dye forming coupler has the structure: wherein:
R₆ is hydrogen or a substituent;
R₇ is a ballast group; and
X is hydrogen or a coupling-off-group.

4. A photographic element of claim 3, wherein R₆ is a t-alkyl group.

5. A photographic element of claim 1, wherein in compound N:
each of W², W³, W⁴, W⁵, W⁶ and W⁷ is hydrogen, alkyl or alkoxy having no more than 20 carbon atoms.

6. A photographic element of claim 1, wherein compound N has a structure selected from: and

7. A photographic element of claim 1, wherein compound S has the structure: wherein:
R₈ represents alkyl, alkoxy, alkylthio, amido, ureido, or halogen;
R₉ is alkyl;
r is an integer of 1 or 2; and
s is an integer of 0 to 4; and
compound R has the structure: wherein
each R₁ independently is hydrogen, alkyl or cycloalkyl of 1 to 8 carbon atoms;
each R₂ is independently hydrogen, hydroxy, alkyl or alkoxy of 1 to 8 carbon atoms;
each m is an integers of 0 to 2; and
A is an alkylene group of 1 to 10 carbon atoms.

8. A photographic element of claim 1, wherein each of compounds R and S are present in a range of about 0.2 to 2.0 moles compound per mole magenta dye forming coupler and comopund N is present in a range of about 0.01 to 0.5 moles compound per mole magenta dye forming coupler.

9. A photographic element of claim 9, further comprising a phthalate ester coupler solvent.

10. A photographic element of claim 1, wherein the support is opaque.
